

# United States Patent Office.

JOHN CORSON, OF WASHINGTON, DISTRICT OF COLUMBIA, ASSIGNOR TO  
HIMSELF AND DANIEL BREED, OF SAME PLACE.

*Letters Patent No. 95,882, dated October 19, 1869.*

## IMPROVEMENT IN THE MANUFACTURE AND PRESERVATION OF METALS.

The Schedule referred to in these Letters Patent and making part of the same.

*To all whom it may concern:*

Be it known that I, JOHN CORSON, of Washington, in the county of Washington, and District of Columbia, have invented a new and useful Improvement in the Manufacture and Preservation of Metals; and I do hereby declare that the following is a full and exact description thereof.

My invention consists in manufacturing, tempering, and preserving metals in a state of insulation from earth-currents of electricity, in order to prevent crystallization, and to produce and retain the metal in a superior fibrous condition.

In the practical application of my invention, it is necessary to insulate the foundation of the furnace, the hammers, anvils, floors for the workmen, furnace-tools, rollers and machinery, moulds; forges, and all appliances for working metals and tempering edge-tools, store-houses and racks where metals are kept, and every place and thing in contact or connection with the metal. Also, railroads, bridges, buildings, and other structures made of iron, in whole or in part, should be insulated.

For the purpose of insulation, glass tiles, balls, pillars, or any other suitable means may be employed. Upon railroads a board of gutta-percha, or other bad conductor may be placed between the ties and rails,

and also under the chairs, or under the rails, upon the chairs, thus forming an insulating, elastic cushion for the rails, and thereby preventing the usually severe concussion of the rolling stock. Or other means of insulation may be employed.

My invention may be applied not only to iron and steel, but also to copper, brass, and other metals and alloys where it is desirable to secure a highly fibrous condition, and prevent or retard crystallization.

I do not limit my invention to the above-described details, as other equivalent means may be employed without departing from my invention.

Having described my invention,  
I claim the above-described mode of manufacturing working, tempering, storing, and preserving metals in a state of insulation from earth-currents of electricity, in order to produce and preserve a superior fibrous condition of the metal, and to prevent or retard the crystallization and deterioration of the same, using the aforesaid means, or their equivalents, involving the same principles, substantially as set forth.

JOHN CORSON.

Witnesses:

DANIEL BREED,  
EDM. F. BROWN.